

## UNITED STATES PATENT OFFICE

ROBERT E. WILLARD, OF MINNEAPOLIS, MINNESOTA, ASSIGNOR TO THE BRIQUET ENGINEERING COMPANY, OF MINNEAPOLIS, MINNESOTA, A CORPORATION OF DELAWARE

## BINDER AND BRIQUETTE AND PROCESS OF PRODUCING SAME

No Drawing.

Application filed June 22, 1929. Serial No. 373,057.

This invention relates to the making first, of an improved briquette binder, and second, to the making of an improved briquette, and the invention includes not only the said materials as new articles of manufacture but also the processes or methods by which they are produced. The binder is made by commingling sulphur, preferably ground but not to the fineness of flour, with heated asphalt, preferably of the grade commonly used for binders in the briquetting industry. The briquette is then formed by commingling the binder with ground coal which is at a quite high temperature, but at a temperature less than that which will carry off the volatile substances of the coal, and subsequently forming the briquette under high compression.

In practice, I have found that when approximately twenty per cent of ground sulphur is added to asphalt having a melting point of 185° F., the melting point of the mixture is reduced from 185° to approximately 152° F.; that the temperature at which the binder volatiles are released is reduced about twenty-five per cent; and that the elasticity of the binder is increased about one hundred per cent. This percentage of change holds good with a sulphur content of from ten to twenty per cent. Also I have found that the sulphur thus added to the asphalt causes certain chemical reactions that materially alter the characteristics of the asphalt and produce a binder with all of the qualities required in an efficient briquette binder and make possible a superior briquette.

It is a recognized fact that a certain portion of the sulphur is absorbed into the molecules of the asphalt and is given off in the form of gas at a temperature under the temperature required to distill the coal of the briquette, but the exact nature of the chemical actions that take place I have not been able to determine at the present time. The sulphur seems to act as a catalyst which causes the production of a superior briquette binder by causing chemical reactions or physical changes into which the sulphur does not directly enter.

The following is one example of an effi-

cient way that I have, in practice, practically carried out my invention.

In preparing the binder, eighty-five parts of standard grade binder asphalt having a melting point of 185° F., was heated to a temperature of approximately 200° F., and to this was added fifteen parts of ground sulphur, the liquid being then thoroughly commingled and aerated. Virginia anthracite coal mined from the Langhorne seam near Pulaski, Virginia, which has a volatile content of about eleven per cent, was ground to pass a sixteen mesh screen and was raised to a temperature of approximately 450° F. To approximately ninety-five parts of this ground coal cooled to approximately the temperature of 350° F., five parts of the prepared binder was added while the temperature of the mixture was approximately 350° F. The coal thoroughly mixed with the binder was then run through coolers and the temperature was brought down to approximately 160° F. and at approximately this latter noted temperature, the material was passed to the press and the briquettes then formed under high compression.

The briquettes thus produced were found to be of very high heat-producing efficiency and having all the qualities desirable in superior briquettes. These briquettes burn practically smokeless. They form a hard compact coke at the least possible temperature that will hold the particles of coal together and prevent disintegration of the briquette during combustion. The volatiles of the binder are released at lower temperature than the volatile of the coal from which the briquettes are made and consequently the coal volatiles are ignited and completely consumed with elimination of smoke. Also the binder gives the briquette increased elasticity and strength which prevents breakage and deterioration of the briquette during shipment and storage.

I have found that the percentage of sulphur required in the binder and the temperature to which the binder must be subject before being commingled with the coal is governed very considerably by the volatile content of the coal used and the tempera-

55

60

65

70

75

80

85

90

95

100

ture at which the volatile of the coal will be released. As a general rule, the higher the volatile content of the coal and the lower the temperature of distillation, the more sulphur and the higher temperature required to produce the binder. By heating ground coal to a temperature that just begins to soften the coal tar content, but not to a point that will carry off the volatile of the coal, I have been able to use as much as two per cent less binder to produce a satisfactory briquette. The temperatures mentioned are considerably above those usually employed for producing briquettes, but I have found such temperatures desirable in carrying out my invention.

The following is an example of the manner in which I have successfully carried out my invention in making briquettes from bituminous coal from Williamson County, Illinois, which coal has a volatile content of approximately thirty-eight per cent. In preparing the binder for this type of briquette, I used seventy-five parts of standard binder asphalt having a melting point of 185° F., brought the same to a temperature of approximately 250° F., I then added twenty-five parts of ground sulphur and thoroughly agitated and mixed the same. Then to approximately ninety-three parts of said bituminous coal ground so as to pass through 16 mesh screen, I added seven parts of said binder and thoroughly commingled the same while at a temperature of approximately 300° F. The mixture was then reduced in temperature to approximately 160° F. and delivered to the press for the formation of the briquette. This produced a hard waterproof briquette which during the combustion will not disintegrate and will not produce smoke except possibly for a few minutes during ignition and will not produce soot and will retain form until completely consumed. The briquettes burn with a medium length bright blue-white flame.

From what has been said, it will be understood that the temperatures required and proportions of materials will vary for different kinds of coal or briquette-producing substances. In a general way, I have found that the temperatures to which the ground coal should be raised before commingling the binder therewith will vary from 200 to 450° F. and that the temperatures to which the binder should be raised before being commingled with the coal vary from 200 to 325° F.

The term "ground coal" is herein used to include ground lignite.

What I claim is:

1. The process of making briquettes which consists in mixing together liquid asphalt and sulphur and dissolving the sulphur into the asphalt and in thereafter commingling the resulting binder with ground briquette

material at a temperature exceeding the melting point of the asphalt, but not high enough to carry off the volatile substance of the briquette material.

2. The process of making briquettes which consists in mixing together liquid asphalt and sulphur and dissolving the sulphur in the asphalt and in thereafter commingling the resulting binder with ground briquette material at a temperature exceeding the melting point of the asphalt, but not high enough to carry off the volatile substances of the briquette material, and in thereafter cooling the mixture to a temperature much lower than the temperature at which the binder was commingled with the briquette material and subjecting the cooled mixture to a briquette press.

In testimony whereof I affix my signature.

ROBERT E. WILLARD. 85

70

75

80

85

90

95

100

105

110

115

120

125

130